# EUROPEAN PATENT SPECIFICATION

(11) **EP 2 341 154 B1**
(45) Date of publication and mention of the grant of the patent: **25.02.2015**
(21) Application number: 10382002.3
(22) Date of filing: 05.01.2010
(51) Int. Cl.: C21C 1/10

(54) **Process for making nodular cast iron**
Verfahren zur Herstellung von Gusseisen mit Kugelgraphit
Procédé de production de fonte nodulaire

(43) Date of publication of application: 06.07.2011
(73) Proprietor: Fernandez Teran, Pedro, 08400 Barcelona (ES)
(72) Inventor: Fernandez Teran, Pedro, 08400 Barcelona (ES)
(74) Representative: Carpintero Lopez, Francisco

(56) References cited:
- GB-A- 1 527 054
- JP-A- 61 119 351
- US-A- 2 855 336
- US-A- 4 252 559
- US-A- 5 758 706

## Description

### Technical Field of the Invention

The invention starts from the use of a metal chilled casting installation, with a further annealing heat treatment, which produces ferritic flake graphite gray cast iron.

The object of the present invention is a process which allows obtaining ferritic-perlitic nodular gray cast iron in the as-cast condition in a metal chill-mold (without heat treatment) in one and the same casting installation which produces ferritic flake graphite gray cast iron.

An embodiment variant provides obtaining in parallel nodular gray cast iron in metal chill-mold and flake graphite gray cast iron, starting from a common load in the melting furnace.

### Background of the Invention

Normally, the foundries are specialized in flake graphite type or nodular type casting. Thus, when they are required to produce the two casting qualities due to certain circumstances, it is necessary to separate the materials and the material transfer and casting elements, among other modifications of the foundry.

From another point of view, due the risks of contamination of some materials with others, it is necessary to perform the casting of one type of material before the other and that the returns (sprues, risers, defective parts, etc.) do not mix with the other type of material, i.e., it is not possible to melt the two types of materials at the same time or simultaneously. As a result, the raw material collections are extensive and require very strict controls.

US Patent 2 855 336 discloses a method for obtaining centrifugated tubing in steel molds of white cast (cementite), therfore the tubing should be treated in an annealing oven in order to produce nodular structure in the product.

US Patent 4 252 559 discloses the use of an electric arc furnace in order to obtain base cast iron. The carbon content of the cast iron can be brought to the desired value by adding carburizing agents in the furnace. In this regard, it is important mentioning that the main object of a foundry is to obtain cast products, this document of the prior art only makes improvements in only one equipment of the foundry. The problem of producing both casting qualities using the same equipments of a foundry is not disclosed.

GB Patent 1 527 054 discloses an automatic treatment system wherein inoculation is carry out with Fe Si Mg and inoculants in the melted material in order to obtain nodular cast, the inoculation is carry out at temperatures of 1380°C to 1430° C. The inoculation step is performed during pouring and not by the addition inoculants into the ladle.

The most currently used and common nodular casting process is the so-called *disamatic*®, in which green sand molds are used without metal cases, and the molding is carried out under high pressure. There are others such as molding with chemical setting, but the *disamatic*® system is preferably used for the automotive industry and more specifically for manufacturing several components of vehicle brake systems.

This nodular casting process produces very high quality parts for many sectors of the industry in general and particularly for the automotive sector, for example, the nodular casting allows obtaining parts for disc brakes (actuators) the components of which are clamps and forks. Likewise, brake parts such as the controls (master cylinders, wheel cylinders, compensators and clutch controls) have always been mainly cast in a metal chill-mold.

The casting parts for brake systems and, therefore, for safety systems need to have a series of characteristics which must be met to give the guarantees which are required by automobile manufacturers, ranging from the service, quality and price to the quickness in the development of new products at the lowest costs. Evidently, brake manufacturers require the same from the foundries that manufacture these parts.

The main characteristics in the parts that brake manufacturers require from foundries, in addition to the mechanical characteristics such as tensile strength, elastic limit, elongation, hardness, resilience and type of structure, are: the parts must be easy to machine, have a good machining surface finish, less wear of the tools when machining, the material must be very compact and have good leak-tightness, dimensional stability before and after machining, the parts must have a high capacity of thermal evacuation, and the material to be machined must be the minimal amount due to reduced tolerances.

With respect to the casting process, brake manufacturers require: that it has a good internal quality by a controlled variable process, that it has a high productivity, without intermediate stocks, that the lead time is the lowest possible, that the costs are very competitive and that the release of new products is very fast.

The foundries specialized in producing flake graphite gray cast iron in metal chill-mold have an increasingly more limited field in industrial sectors, such as the automotive and wind sectors, where parts of both qualities are required i.e., flake graphite gray cast iron and nodular gray cast iron quality. This is why the applicant of the present application, who is aware of the drawbacks and has ample experience in the field of casting, applies knowledge, research and innovation to developing a process which allows using, without needing structural changes, expansions and/or adaptations, a conventional flake graphite gray cast iron in metal chill-mold installation to also obtain nodular gray cast iron and even both qualities in parallel.

A flake graphite gray cast iron in metal chill-mold installation has at least one melting furnace, and its corresponding loader; at least one maintenance furnace; a transfer ladle for transferring the molten load from the melting furnace to the maintenance furnace; a distribution ladle for feeding the casting ladle; a carousel with a plurality of metal molds (chill-molds) in which the hot melt is cast; feeding and classification belts and an annealing heat treatment furnace.

The process for producing flake graphite gray cast iron in metal chill-mold, when only this type of quality is produced, is as follows:

A loader feeds the metal and non-metal load to the melting furnace and when the metal is molten, with an equivalent carbon content of 4.40 to 4.60%, it is transferred to the maintenance furnace by means of the transfer ladle.

In the maintenance furnace, the composition and the temperature are adjusted. The molten load is passed from the maintenance furnace to the distribution ladle and from the latter to the casting ladle.

The casting ladle casts the cast iron in the molds and when the parts have solidified they are demolded.

The demolded parts are transported to the heat treatment furnace and from the latter to the different phases of the process of classification, unitary control and finishing.

### Object of the Invention

The invention which is the object of this application is based on a conventional installation, such as the one described above and based

### Description of the Invention

The process object of the present application, i.e., the process for obtaining nodular gray cast iron in metal chill-mold in the as-cast condition, comprises the following steps:

Feeding the melting furnace with a metal and non-metal load, to obtain an equivalent carbon content of 4.70 to 4.90 and transferring the load to the maintenance furnace by means of the transfer ladle.

In the maintenance furnace, the metal base is completely refined in terms of composition and temperature. When the base metal is correct, it is treated with Fe-Si-Mg and inoculant in the distribution ladle itself and then an additional amount of inoculant is added into the casting stream in the casting ladle.

Fe-Si-Mg is the nodulizing agent and 7 to 10% by weight of the load to be treated is added. The inoculant which is added together with Fe-Si-Mg is to reduce the formation of metal carbides (cementite) of the latter and to increase the power of nucleation (nodularization) at the time of the treatment. The amount of inoculant which is added in the distribution ladle is 0.15 to 0.22% the weight of the load.

The inoculant which is added into the casting stream in the casting ladle is to reinforce the non-precipitation of cementite due to the quick solidification of the metal in the chill-mold. This addition of inoculant into the casting stream in the casting ladle is 0.07 to 0.15%.

It is cast from the casting ladle into the metal molds and when the parts have solidified they are demolded and passed to containers in order to clean them, classify them and perform the unitary controls and carry out the finishing operations when they are cold.

In some cases, the parts with very special characteristics are passed through the heat treatment (ferritization) furnace to improve their strength and elongation values. Furthermore, the subsequent heat treatment gives a very special characteristic to the parts produced in metal chill-mold in terms of the absorption of noises caused by friction or contact with other parts (vibrations due to friction).

A variant of the invention provides a process which allows obtaining in parallel nodular gray cast iron and flake graphite cast iron in metal chill-mold, for which a metal and non-metal load is initially fed to a melting furnace.

The material of the melting furnace is transferred from the melting due to friction).

A variant of the invention provides a process which allows obtaining in parallel nodular gray cast iron and flake graphite cast iron in metal chill-mold, for which a metal and non-metal load is initially fed to a melting furnace.

The material of the melting furnace is transferred from the melting furnace both to a first maintenance furnace (for the flake graphite cast iron) and to a second maintenance furnace (for the nodular cast iron) by means of a transfer ladle.

However, in the event of producing flake graphite cast iron, FeP and FeMn are added in the transfer ladle and the material is poured into the first maintenance furnace.

And in the event of producing nodular cast iron, graphite, FeSi and FeMn are added in the transfer ladle and the material is poured into the second maintenance furnace.

Subsequently, the material is poured from the first maintenance furnace and from the second maintenance furnace to at least one distribution ladle; in which, in the event of producing nodular cast iron a nodulizing agent and an inoculant are added in the distribution ladle. And for the case of flake graphite cast iron no component is added.

The material is fed from the distribution ladle to at least one casting ladle, in which in the event of producing nodular cast iron an additional amount of inoculant is added in the casting ladle. For the case of flake graphite cast iron no component is added.

Finally, the material from the casting ladle is poured into at least one metal mold.

For the process of simultaneously obtaining nodular and flake graphite cast iron, the equivalent carbon content in the melting furnace is 4.4 to 4.60, for the purpose of allowing producing both types of cast irons.

In an additional embodiment, after adding the graphite, FeSi and FeMn in the transfer ladle for the nodular cast iron, a molten material with the following composition is obtained:
3.90-4.00% C;
2.60-2.80% Si;
0.65-0.70% Mn;
0.010-0.015% S and
0.10- 0.15% P.

Likewise, for the flake graphite cast iron, after adding FeP and FeMn, a molten material with the following composition is obtained:
3.57-3.62% C;
2.40- 2.50% Si;
0.60-0.70% Mn;
0.010-0.015% S and
0.30-0.35% P.

In the variant of the process for obtaining the two types of cast irons, for the purpose of preventing down times and optimizing the flow of materials, it is preferable to work with two maintenance furnaces and two carousels of metal molds. The melting furnace can be the same but it is more operative to use one of the melting furnaces for the flow of materials of the flake graphite gray cast iron and a second maintenance furnace for the flow of materials of the nodular gray cast iron.

### Brief Description of the Drawings

To complement the description which is being made and for the purpose of aiding to better understand the features of the invention according to certain preferred practical embodiments thereof, a set of drawings is attached as an integral part of this description, in which the following has been depicted with an illustrative and non-limiting character:
Figure 1 schematically depicts a conventional type of installation for flake graphite cast iron production, in which the flow of materials has been indicated by means of arrows.
Figure 2 depicts the same diagram of the previous figure, in which the flow of materials has been indicated with arrows and the points at which the additives (nodulizing agent and inoculant) are added have been indicated with a circle.
Figure 3 depicts the same previous diagram in which the flow of materials for nodular cast iron has been indicated with solid arrows and the flow of materials for flake graphite cast iron has been indicated with dotted arrows, and the points at which the additives are added have been indicated with a circle.

### Detailed Description of the Preferred Embodiments of the Invention

As has been mentioned, the present invention provides a process for making nodular cast iron using a prior art installation which is traditionally intended for flake graphite cast iron, which is described below.

### Flake graphite cast iron

To contextualize the above, reference is made to Figure 1, which shows a traditional casting installation 10 formed by a melting furnace 20 in which a casting load introduced by a feeding belt 11 is melted. In this installation 10 there is also a transfer ladle 30 which receives the material from the melting furnace 20. Another part of this installation is a maintenance furnace 40 which is fed by the transfer ladle 30. In the installation 10, a distribution ladle 50 receives the material from the maintenance furnace 40 and feeds it to at least one casting ladle 60; from which the molten material is drained towards at least one metal mold 70 assembled in a carousel 80.

Once the parts have solidified, they are demolded and transported by means of a conveyor belt 12 and a classification belt 13 towards a heat treatment furnace 90 and from the latter to the different phases of the process of classification, unitary control and finishing. The returns are recovered at the outlet 95.

More particularly, to make the flake graphite cast iron the (metal and non-metal) casting load is fed to the melting furnace 20, when the metal is molten and an equivalent carbon content "Ce" of 4.40 to 4.60 has been achieved, the molten material is transferred to the maintenance furnace 40 by means of the transfer ladle 30, and there the composition and the temperature of the molten material are adjusted in the event that there is any deviation.

In a typical example of this type of flake graphite cast iron, the casting load comprises as metal materials: pig iron, first quality scraps, internal returns, graphite, FeSi, FeP and FeMn, achieving a composition of:
3.57-3.62% C;
2.40-2.50% Si;
0.60-0.70% Mn:
0.010-0.015% S and
0.30-0.35% P.

In turn, when the molten material reaches the maintenance furnace 40 its composition is the same as that present in the melting furnace 20, with some small adjustments if there is a deviation. Likewise, the same composition as the one of the maintenance furnace 40 is in the distribution ladle 50 and casting ladle 60.

Having described this installation, the way in which it is used to the aid of Figure 2 has been devised.

In the process, a casting load is fed by means of a conveyor belt 11 to a melting furnace 20; this casting load is then transferred to a maintenance furnace 40 by means of a transfer ladle 30.

The molten material is poured from the maintenance furnace 40 into a distribution ladle 50, adding thereto a nodulizing agent and an inoculant. The distribution ladle 50 is marked in Figure 2 by means of a circle with a dotted line to indicate that that is where the nodulizing agent and the inoculant are added, establishing a great difference with the prior art.

The distribution ladle 50 feeds the molten material to at least one casting ladle 60, in which an additional amount of inoculant is added; and, finally, the molten material is cast from the casting ladle 60 into metal molds 70 assembled in a carousel. Again, a circle with a dotted line is used to indicate that an additional amount of inoculant is added in the casting ladle 60.

In a preferred embodiment of this process, it is preferred that the equivalent carbon content in the melting furnace 20 is 4.7 to 4.90 to be able to obtain the nodular cast iron in the installation 10.

The casting load used for this process comprises: pig iron, first quality scraps, internal returns, graphite, FeSi and FeMn. In the maintenance furnace 40 this molten material is completely adjusted in terms of composition and temperature.

When the molten material has a correct composition and temperature, it is treated with the nodulizing agent and the inoculant in the distribution ladle 50. The nodulizing agent used is preferably Fe-Si-Mg and is added in a percentage of 7 to 10% with respect to the molten material to be treated. The inoculant which is added together with the nodulizing agent is to reduce the power of formation and precipitation of metal carbides (cementite) due to the quick solidification of the metal in the chill-mold and to increase the power of nucleation (nodularization) at the time of the treatment. The inoculant used is preferably of the Germalloy type with a composition of 71.50% Si; 0.88% Ca and 3.78% Al and is added in a percentage of 0.15 to 0.22 with respect to the molten material to be treated.

An oxidizing reaction and at the same time an increase of the Si due to the FeSi content in the alloy occur in the distribution ladle 50, after the treatment with the nodulizing agent and the inoculant. molten material to be treated.

An oxidizing reaction and at the same time an increase of the Si due to the FeSi content in the alloy occur in the distribution ladle 50, after the treatment with the nodulizing agent and the inoculant.

After the treatment with the nodulizing agent and the inoculant, the molten material has the following composition in the distribution ladle 50:
3.60-3.80% C;
2.80-3.00% Si;
0.65-0.75% Mn,
0.008-0.013% S; and,
0.10-0.15% P.

The composition of the molten material in the distribution ladle 50 also contains residual Mg, Ti and Cu.

As has been mentioned, an inoculant is added in the casting ladle 60, which inoculant is preferably of the SMW type with the following composition 62.80% Si; 2.35% Ca; 0.97% Al; 0.81% Bi and 0.99% TR.

The inoculant which is added into the casting stream of the casting ladle is to reinforce the non-precipitation of cementite due to the quick solidification of the metal in the chill-mold. This addition of inoculant into the casting stream is carried out in a proportion of 0.07 to 0.15% by weight of the treated load.

As is observed in Figure 3, the molds 70 are assembled in a carousel 80, so that in the moment in which the parts have solidified they are demolded and passed to containers and when the parts have cooled, they are cleaned, classified, unitarily controlled and the finishing operations are carried out.

As is observed, the process of the present invention is characterized by the way in which ferritic-perlitic nodular gray cast iron in the as-cast condition (without heat treatment) is obtained, using the same installation with which the ferritic flake graphite gray cast iron with subsequent annealing heat treatment is produced.

In an embodiment of the process, when parts with very special characteristics are required, the parts are passed through the treatment (ferritization) furnace 90 to improve the strength and elongation values.

It is very important to mention that nodular casting in metal mold allows the produced parts to have advantages with respect to those made according to the prior art (disamatic type green sand, furan resin or chemical setting of the mold, ceramic, precoated sand etc.), the following can be mentioned among said advantages:
- Better machining as a result of the much finer and better distributed graphite nodules which reduce the shearing stresses and this is much more clearly shown when it is treated.
- The fineness and distribution of the graphite nodules also have another advantage over the quality of the surface finish state in machining: such as: milling, reaming, grinding, burnishing, rolling, boring and threading.
- Its surface finish quality often allows eliminating an obligatory rolling operation in another type of casting.
- It allows working at higher shearing speeds and the wear of tools is much lower, therefore the machining times and the stops for changing tools are reduced, which allows considerable productivity increases (in some cases productivity increases of 50% can be reached).
- Greater tightness since its hypereutectic composition causes a grain expansion during the solidification which, due to the rigidity of the mold, only allows doing it towards the interior, which causes a more compact cast iron. The fineness of the graphite nodules reduces the effect of notches, thus improving the resistance to pressure and also the fatigue strength.
- The metal mold furthermore allows a much greater reproducibility.

Other also very important properties which are obtained by means of casting in metal chill-mold are: the thermal evacuation capacity as a result of the well distributed and fine-grain structure, the reduction of the size tolerances due to the resistance of the metal mold during solidification, the possibility of reducing allowance or overthicknesses for machining due to its high stability and the reproducibility of the molds, as well as the capacity to produce small parts.

In addition to all that mentioned above, this type of part obtained by means of casting in metal chill-mold allows, for their structural characteristics with a subsequent treatment, acoustic absorption or non-amplification of noises just like compact graphite but with much better mechanical characteristics.

Another aspect of the present invention is described below.

### Parallel flake graphite and nodular cast

In an embodiment variant, the process allows obtaining in parallel flake graphite and nodular cast iron, to that end reference is made to Figure 3, which shows a casting installation 110 similar to the one described for obtaining flake graphite in a conventional manner but in which, to make it more operative and profitable, using the times better, two melting furnaces, two maintenance furnace and two carousels of metal molds are used. For a better understanding of the installation 110, its common elements with respect to the installation of Figures 1 and 2 have the same reference numbers. In Figure 3 the flow of materials for nodular cast iron are marked with a solid line and for flake graphite cast iron they are marked with a dotted line.

In this casting installation 110 there is a melting furnace 20 for melting a casting load, a parallel melting furnace 20' for providing versatility to the process is also observed. In the casting installation there is also a transfer ladle 30 which receives the material of any of the melting furnaces 20 or 20'. It is also seen that there is a first maintenance furnace 40 and a parallel second maintenance furnace 40', both fed by the transfer ladle 30, the objective of each of these melting furnaces will be explained below. Likewise, a distribution ladle 50 which receives the material from the first maintenance furnace 40 or from the parallel second maintenance furnace 40' is seen in the installation.

In the installation there are also casting ladles 60 and 60' which are fed by the distribution ladle 50; and, finally, at least metal molds 70 assembled in carousels 80 and 80' in which the material is discharged from the casting ladle 60 or 60' are seen. The installation 110 also has a heat treatment furnace 90.

For the process of the present invention, a casting load is fed to the melting furnace 20 or 20'; the material from the melting furnace 20 is then transferred to a first maintenance furnace 40 (for the flake graphite cast iron) and to a second maintenance furnace 40' (for the nodular cast iron) by means of a transfer ladle 30, in which, in the event of producing flake graphite cast iron, FeP and FeMn are added in the transfer ladle 30, and poured into the maintenance furnace 40; and, in the event of producing nodular cast iron, graphite, FeSi and FeMn are added in the transfer ladle, and the material is poured into the parallel maintenance furnace 40'. The transfer ladle 30 is marked with a circle to indicate that said addition is carried out therein depending on the type of cast iron to be obtained.

The material is subsequently poured from the first maintenance furnace 40 or from the second maintenance furnace 40' to at least one distribution ladle 50; in which in the event of producing nodular cast iron a nodulizing agent and an inoculant are added to the distribution ladle 50. For the case of flake graphite cast iron no component is added.

Then, in the event of producing nodular cast iron an additional amount of inoculant is added in the casting ladle 60' whereas no component is added in the casting ladle 60 for flake graphite cast iron.

However, in this simultaneous process for obtaining both types of cast irons, the casting load comprises: pig iron, first quality scraps, internal returns, graphite and FeSi, achieving an equivalent carbon content in the melting furnace 20 or 20' of 4.4 to 4.60. In other words, one and the same load is used whether one type or another of cast iron is to be produced.

As has been described, the changes necessary for achieving one type of cast iron or another are done below. For the case of nodular cast iron, after adding graphite, Fe-Si and Fe-Mn in the transfer ladle 30, a molten material with the following composition is obtained:
3.90-4.00% C;
2.60-2.80% Si;
0.65-0.70% Mn;
0.010-0.015% S and
0.10- 0.15% P.

in the distribution ladle, Fe-Si-Mg is added as nodulizing agent and the inoculant is of the germalloy type with a composition of 71.50% Si; 0.88% Ca and 3.78% Al and is added in a percentage of 0.15 to 0.22 with respect to the molten material to be treated.

The composition of the molten material in the distribution ladle 50 for nodular cast iron is:
3.60-3.80% C;
2.80-3.00% Si;
0.65-0.75% Mn,
0.008-0.013% S and
0.10-0.15% P,

The molten material also contains residual Mg, Ti and Cu in the distribution ladle 50.

With respect to flake graphite cast iron, after adding FeP and FeMn in the transfer ladle 30, a molten material with the following composition is obtained:
3.57-3.62% C;
2.40- 2.50% Si;
0.60-0.70% Mn;
0.010-0.015% S and
0.30-0.35% P.

The composition achieved in the transfer ladle 30 with a phosphorus content of 0.30-0.35% allows increasing the castability and the manganese content neutralizes the action of the sulfur. After that the process is the same as that shown in Figure 1, i.e., the molten material from the maintenance furnace 40 passes to the distribution ladle 50 and from there to the casting ladle 60 to pour the molten material into the mold 70.

A very important aspect in the present invention relates to the metal molds used compared to the casting in any of the known types (disamatic type green sand, furan resin or chemical setting of the mold, ceramic, precoated sand etc.), since their specific properties are directly linked to their metallurgic structure and to the mode of preparation.

The process for obtaining nodular cast iron in the as-cast condition and in metal mold (chill-mold) has a series of advantages compared to the traditional disamatic sand process, including the following:
- The lead time passes from one day to two and a half hours.
- Evidently upon reducing the lead time, the control of the process is much easier and quicker and will therefore produce parts of a better quality.
- The process for manufacturing prototypes for new products passes from one month to one week.
- There are no intermediate stocks.
- Lower percentage of rejected parts due to the reduced lead time and furthermore without intermediate stocks.
- Capacity to produce smaller batches.
- Capacity to simultaneously cast 36 different parts.
- Better service due to: shorter lead time, without intermediate stocks, better control of the process, lower internal rejection, capacity for small batches, simultaneous manufacture of different references and greater quickness in the launch of new products.

Likewise, in an overall manner this installation which allows the simultaneous casting of both cast iron qualities has the following advantages:
- the same metal load quality.
- the same ferroalloys.
- the same melting furnaces.
- the same maintenance furnaces.
- the same distribution ladles.
- the same casting ladles.
- the same casting carousels
- the same casting chill-molds, with different references
- the same belts for discharging parts which have been completely cast.

In view of this description and set of figures, the person skilled in the art will understand that the embodiments of the invention which have been described can be combined in many ways within the object of the invention.

## Claims

1. Process for obtaining nodular gray cast iron as cast in metal chill-mold in one and the same casting installation which produces ferritic flake graphite gray cast iron, the installation consists of:
- at least one melting furnace (20)
- at least one maintenance furnace (40)
- at least one transfer ladle (30) for transferring the molten load from the melting furnace (20) to the maintenance furnace (40)
- at least one distribution ladle (50) for passing the loads of the melting furnaces to the casting ladle
- at least one casting ladle (60) fed by the distribution ladle (50)
- at least one carousel (80) with at least one metal chill-mold (70) in which the material is discharged from the casting ladle (60) **characterized in that** it comprises the steps of:
a) feeding a casting load to the melting furnace (20); wherein, the equivalent carbon content in the melting furnace is 4.7 to 4.90;
b) transferring the molten material from the melting furnace (20) to the maintenance furnace (40) by means of the transfer ladle (30);
c) pouring the material from the maintenance furnace in the distribution ladle (50) adding thereto a nodulizing agent and an inoculant; so that after the treatment with the inoculant and the nodulizing agent, the molten material in the distribution ladle (50) has the following composition:
3.60-3.80% C;
2.80-3.00% Si;
0.65-0.75% Mn,
0.008-0.013% S and
0.10-0.15% P;
d) feeding said at least one casting ladle (60) with the material from the distribution ladle (50), wherein an additional amount of inoculant is added in the casting ladle (60);
e) casting the material from the casting ladle (60) in said at least one a metal chill-mold (70) by gravity; and
f) cooling and demolding the part once solidified.

2. Process for obtaining nodular gray cast iron in metal chill-mold according to claim 1, **characterized in that** the casting load comprises:
pig iron, first quality scraps, internal returns, graphite, FeSi and FeMn.

3. Process for obtaining nodular gray cast iron in metal chill-mold according to any of claims 1 or 2, **characterized in that** the nodulizing agent is Fe-Si-Mg and is added in a percentage of 7 to 10% with respect to the weight of the molten material to be treated.

4. Process for obtaining nodular gray cast iron in metal chill-mold according to any of claims 1 to 3, **characterized in that** the inoculant added in the distribution ladle (50) is of the Germalloy type with a composition of 71.50% Si; 0.88% Ca and 3.78% Al and is added in a percentage of 0.15 to 0.22 with respect to the molten material to be treated.

5. Process for obtaining nodular gray cast iron in metal chill-mold according to any of claims 1 to 4, **characterized in that** the inoculant which is added into the casting stream in the casting ladle (60) is of the SMW type with the following composition 62.80% Si; 2.35% Ca; 0.97% Al; 0.81% Bi and 0.99% TR and is added in the amount of 0.07 to 0.15% by weight of the load.

6. Process for obtaining nodular gray cast iron in metal chill-mold according to any of claims 1- 5, **characterized in that** the produced piece is fed to a treatment furnance (90) in order to improve the strength and elongation.

## Patentansprüche

1. Verfahren zur Herstellung von Gusseisen mit Kugelgraphit als Guss in Metall-Kokille in ein und derselben Guss-Installation, welche Gusseisen mit ferritischem Lamellengraphit herstellt, die Installation besteht aus:
- mindestens einem Schmelzofen (20)
- mindestens einem Instandhaltungsofen (40)
- mindestens einer Transportpfanne (30) um die geschmolzene Masse von dem Schmelzofen (20) zum Erhaltungsofen (40) zu transferieren
- mindestens ein Verteilergefäß (50) um die Masse des Schmelzofens zur Gießpfanne weiterzugeben
- mindestens eine Gießpfanne (60) gespeist durch das Verteilergefäß (50)
- mindestens ein Umlaufförderer (80) mit mindestens einer Metall-Kokille (70) in welche das Material von der Gießpfanne (60) entladen wird,
**dadurch gekennzeichnet,**
**dass** es folgende Schritte umfasst:
a) Speisen eines Schmelzofens (20) mit einer Gieß-Masse; wobei der entsprechende Kohlenstoff-Gehalt im Schmelzofen 4.7 bis 4.90 beträgt;
b) Transferieren des geschmolzenen Materials von dem Schmelzofen (20) zum Instandhaltungsofen (40) mittels der Transportpfanne (30);
c) Gießen des Materials aus dem Instandhaltungsofen in das Verteilergefäß (50), dazu gebend ein Agglomerations-Agens und ein Impfmittel; so dass nach der Behandlung mit dem Impfmittel und dem Agglomerations-Agens das geschmolzene Material in dem Verteilergefäß (50) folgende Zusammensetzung hat:
3,60-3,80% C;
2,80-3,00% Si;
0,65-0,75% Mn;
0,008-0,013% S und
0,10-0,15% P;
d) Speisen der mindestens einen Gießpfanne (60) mit dem Material aus dem Verteilergefäß (50) wobei eine zusätzliche Menge des Impfmittels der Gießpfanne (60) zugeführt wird;
e) Gießen des Materials aus der Gießpfanne (60) in die mindestens eine Metall-Kokille (70) durch Schwerkraft; und
f) Kühlen und Entformen des Teils sobald es erstarrt ist.

2. Verfahren zur Herstellung von Gusseisen mit Kugelgraphit in Metall-Kokille gemäß Anspruch 1,
**dadurch gekennzeichnet,**
**dass** die Gieß-Masse umfasst:
Roheisen, Überreste erster Qualität, interner Rücklauf, Graphit, FeSi und FeMn.

3. Verfahren zur Herstellung von Gusseisen mit Kugelgraphit in Metall-Kokille gemäß der Ansprüche 1 oder 2,
**dadurch gekennzeichnet,**
**dass** das Agglomerations-Agens Fe-Si-Mg ist und in einem Prozentsatz von 7 bis 10% zugefügt wird in Abhängigkeit des Gewichts des geschmolzenen Materials, das behandelt wird.

4. Verfahren zur Herstellung von Gusseisen mit Kugelgraphit in Metall-Kokille gemäß einem der Ansprüche 1 bis 3,
**dadurch gekennzeichnet,**
**dass** das Impfmittel welches in das Verteilergefäß (50) gegeben wird vom Germalloy-Typ ist mit einer Zusammensetzung von 71,50% Si; 0,88% Ca und 3,78% Al und zugegeben wird mit einem Prozentsatz von 0,15 bis 0,22 in Bezug auf das geschmolzene Material, das behandelt wird.

5. Verfahren zur Herstellung von Gusseisen mit Kugelgraphit in Metall-Kokille gemäß einem der Ansprüche 1 bis 4,
**dadurch gekennzeichnet,**
**dass** das Impfmittel welches in den Gießstrom in der Gießpfanne (60) gegeben wird vom SMW-Typ ist, mit folgender Zusammensetzung 62,80% Si; 2,35% Ca; 0,97% Al; 0,81% Bi und 0,99% TR und in einer Menge von 0,07 bis 0,15% des Gewichts der Masse zugegeben wird.

6. Verfahren zur Herstellung von Gusseisen mit Kugelgraphit in einer Metall-Kokille gemäß einem der Ansprüche 1 bis 5,
**dadurch gekennzeichnet,**
**dass** das produzierte Stück einem Behandlungsofen (90) zugeführt wird um die Stärke und Längung zu verbessern.

## Revendications

1. Procédé pour obtenir une fonte grise nodulaire sous forme coulée dans une lingotière métallique dans une seule et même installation de coulée qui produit de la fonte grise ferritique à graphite lamellaire, l'installation consistant en :
- au moins un four de fusion (20),
- au moins un four de maintien (40),
- au moins une poche de transfert (30) pour transférer la charge fondue du four de fusion (20) au four de maintien (40),
- au moins une poche de distribution (50) pour faire passer les charges des fours de fusion dans la poche de coulée,
- au moins une poche de coulée (60) alimentée par la poche de distribution (50),
- au moins un carrousel (80) ayant au moins une lingotière métallique (70) dans laquelle le matériau est déchargé de la poche de coulée (60),
**caractérisé en ce qu'**il comprend les étapes consistant à :
a) introduire une charge de coulée dans le four de fusion (20) ; l'équivalent en carbone dans le four de fusion étant de 4,7 à 4,90 ;
b) transférer le matériau fondu du four de fusion (20) au four de maintien (40) au moyen de la poche de transfert (30) ;
c) verser le matériau du four de maintien dans la poche de distribution (50) en y ajoutant un agent de nodulisation et un inoculant ; de façon qu'après le traitement avec l'inoculant et l'agent de nodulisation, le matériau fondu dans la poche de distribution (50) ait la composition suivante :
3,60-3,80 % de C ;
2,80-3,00 % de Si ;
0,65-0,75 % de Mn,
0,008-0,013 % de S et
0,10-0,15 % de P ;
d) alimenter ladite au moins une poche de coulée (60) en le matériau provenant de la poche de distribution (50), une quantité additionnelle d'inoculant étant ajoutée dans la poche de coulée (60) ;
e) couler le matériau provenant de la poche de coulée (60) dans ladite au moins une lingotière métallique (70) par gravité ; et
f) refroidir et démouler la pièce une fois solidifiée.

2. Procédé pour obtenir une fonte grise nodulaire dans une lingotière métallique selon la revendication 1, **caractérisé en ce que** la charge de coulée comprend :
de la fonte brute, de la ferraille de première qualité, des déblais internes, du graphite, du FeSi et du FeMn.

3. Procédé pour obtenir une fonte grise nodulaire dans une lingotière métallique selon l'une quelconque des revendications 1 et 2, **caractérisé en ce que** l'agent de nodulisation est Fe-Si-Mg et est ajouté en un pourcentage de 7 à 10 % par rapport au poids du matériau fondu devant être traité.

4. Procédé pour obtenir une fonte grise nodulaire dans une lingotière métallique selon l'une quelconque des revendications 1 à 3, **caractérisé en ce que** l'inoculant ajouté dans la poche de distribution (50) est du type Germalloy avec une composition de 71,50 % de Si ; 0,88 % de Ca et 3,78 % d'Al, et est ajouté en un pourcentage de 0,15 à 0,22 par rapport au matériau fondu devant être traité.

5. Procédé pour obtenir une fonte grise nodulaire dans une lingotière métallique selon l'une quelconque des revendications 1 à 4, **caractérisé en ce que** l'inoculant qui est ajouté dans le courant de coulée dans la poche de coulée (60) est du type SMW avec la composition suivante : 62,80 % de Si ; 2,35 % de Ca ; 0,97 % d'Al ; 0,81 % de Bi et 0,99 % de TR, et est ajouté en une quantité de 0,07 à 0,15 % en poids de la charge.

6. Procédé pour obtenir une fonte grise nodulaire dans une lingotière métallique selon l'une quelconque des revendications 1 à 5, **caractérisé en ce que** la pièce produite est introduite dans un four de traitement (90) destiné à améliorer la résistance et l'allongement.
